

1

3,677,760

## HARDENING PROCESS FOR PHOTOGRAPHIC LIGHT-SENSITIVE ELEMENTS

Haruhiko Iwano and Isao Shimamura, Minami-Ashigaramachi, Kanagawa, Japan, assignors to Fuji Photo Film Co., Ltd., Minami-Ashigara-machi, Kanagawa, Japan  
No Drawing. Filed Apr. 21, 1969, Ser. No. 818,101

Claims priority, application Japan, Apr. 19, 1968,  
43/26,341

Int. Cl. G03c 1/30, 5/26, 5/30

U.S. Cl. 96—50 PT

6 Claims

### ABSTRACT OF THE DISCLOSURE

A process for hardening a silver halide photographic light-sensitive element, which comprises processing the light-sensitive element in a processing bath containing formaldehyde and aromatic dialdehyde represented by the general formula:



wherein R and R' each represents one member selected from the group consisting of a hydrogen atom, a lower alkyl group having 1-5 carbon atoms, and a group capable of increasing water solubility, said group being a member selected from the group consisting of  $\text{SO}_3\text{H}$ ,  $\text{COOH}$ ,  $\text{OH}$  and the  $\text{Na K}$  or  $\text{NH}_4$  salt thereof.

The present invention relates to a process for hardening emulsion layers for silver halide photographic light-sensitive elements.

When a silver halide photographic light-sensitive element is processed at high temperature or it is processed for a long time in solutions of high pH, as is the case with the processing of reversal color photographic materials, it is necessary to harden the emulsion layers thereof at an early stage of the processing to prevent the emulsion layers from being damaged during the processing. The examples of such hardening process are the treatment of photographic materials with an aqueous alkaline solution of an aliphatic aldehyde or with an aqueous solution of aluminum sulfates.

In general, the hardening solution containing an aldehyde harden emulsion layers effectively but their practical applications are limited by the fogging activity of the aldehyde. Therefore, a good hardening solution should have the following features:

(1) The hardening solution should harden emulsion layers effectively without giving chemical fogs to the emulsions. Aldehydes often give fogs to silver halide emulsions owing to their reducing property, therefore, for hardening it is important to overcome such a difficulty.

(2) The hardening solution should afford the quick hardening. That is, the emulsion layers should be hardened within one minute in a pre-hardening bath, or when the hardeners are in developers, they should be hardened quickly at the beginning of the development.

(3) The sufficient hardening should be attained by possibly small content of hardening agent in solution. The benefit of reducing the concentration of hardening agents lies not only in decrease in chemical cost but also in elimination of their undesirable secondary effects and the easier scavenging of residual hardening agents after the pre-hardening process. A large quantity of an aldehyde is necessary for the hardening at low pH. To reduce the aldehyde concentration, the pH of the bath must be increased,

2

which results in the increase in fog formation. Therefore, an improved hardening agent should have a sufficient hardening effect even in solution of low concentration and low pH.

(4) The hardening agent should not react with color-forming materials (couplers) in the emulsion layers.

Therefore, an object of the present invention is to provide a hardening process for photographic light-sensitive elements capable of performing effective hardening without accompanying the aforesaid technical difficulties.

More practically, an object of the present invention is to provide a hardening process for photographic light-sensitive elements capable of exhibiting effectively the hardening effect even at a low concentration of hardening agent in a very short period of time with less formation of fogs and without accompanying undesirable reaction with couplers.

Another object of this invention is to provide a hardening agent capable of being used not only in hardening bath but also in a hardening developer by which hardening is proceeded simultaneously with the course of development.

The inventors have found that the above objects of this invention can be achieved by incorporating formaldehyde and one or more aromatic dialdehydes represented by the following general formula in a processing solution:



wherein R and R' each represents a hydrogen atom, a lower alkyl group such as a methyl group or an ethyl group, a group capable of increasing water-solubility, such as  $\text{—SO}_3\text{H}$ ,  $\text{—COOH}$ , or  $\text{—OH}$ ,  $\text{Na, K}$  or  $\text{NH}_4$  salt thereof.

The typical examples of the aromatic dialdehydes used in the present invention are as follows:

(1) Phthalaldehyde



(2) Isophthalaldehyde



(3) Terephthalaldehyde



(4) 2-methylterephthalaldehyde





An additive amount of the dialdehyde is 0.5-1.5 g. per 55 one liter of the processing solution. And an additive amount of formaldehyde is 5-30 ml. of a 37% aqueous solution per one liter of the processing solution, preferably 20 ml. of a 37% aqueous solution.

Japanese patent publication No. 27,560/64 (U.S. Pat. 60 3,220,849, to Baden and Bard filed Feb. 16, 1962) discloses a process of hardening by a mixture of the above-mentioned dialdehyde and formalin is excellent on the point of less fog formation as compared with the known combination of aldehydes. Furthermore, the combination 65 of this invention is more profitable, because the solution of this combination is more stable and has longer life than the above-mentioned known combination.

Furthermore, since preferable concentration of the dialdehyde for practical hardening is low enough to avoid 70 undesirable secondary effects of the aldehydes, such as increase in fog and side reaction with couplers.

Therefore, the hardening agent of this invention can be used not only for pre-hardener but also for a developer to enable simultaneous hardening and development in one 75 processing bath without much increase in developer fog.

Moreover, the processing bath containing the dialdehyde of this invention may contain inorganic salts such as sodium sulfate, sodium borate, phosphates, pyrophosphates, and a carbonate and also antifoggants such as potassium bromide or potassium iodide.

The invention is explained more in detail by the following examples.

#### EXAMPLE 1

After exposing, a silver halide emulsion layer was subjected to the following photographic processings at 30°C.

| Process:    | Processing time (min.) |
|-------------|------------------------|
| Hardening   | 1                      |
| Washing     | 1                      |
| Development | 4                      |
| Washing     | 0.5                    |
| Fixing      | 1                      |
| Washing     | 1.5                    |

The following eight kinds of hardening compositions were employed.

Composition A: 5.4 ml. of sulfuric acid (1:1), 150 g. of sodium sulfate and 20 g. of sodium acetate; composition B: 5.4 ml. of sulfuric acid, 150 g. of sodium sulfate, 20 g. of sodium acetate, and 20 ml. of formalin (37%); composition C: 5.4 ml. of sulfuric acid, 150 g. of sodium sulfate, 20 g. of sodium acetate, 1.0 g. of phthalaldehyde; composition D: 5.4 ml. of sulfuric acid, 150 g. of sodium sulfate, 20 g. of sodium acetate, and 1.0 g. of isophthalaldehyde; composition E: 5.4 ml. of sulfuric acid, 150 g. of sodium sulfate, 20 g. of sodium acetate, and 1.0 g. of terephthalaldehyde; composition F: 5.4 ml. of sulfuric acid, 150 g. of sodium sulfate, 20 g. of sodium acetate, 1.0 g. of phthalaldehyde, and 20 ml. of formalin (37%); composition G: 5.4 ml. of sulfuric acid, 150 g. of sodium sulfate, 20 g. of sodium acetate, 1.0 g. of isophthalaldehyde, 20 ml. of formalin (37%); composition H: 5.4 ml. of sulfuric acid, 150 g. of sodium sulfate, 20 g. of sodium acetate, 1.0 g. of terephthalaldehyde, and 20 ml. of formalin (37%); composition I: 5.4 ml. of sulfuric acid (1:1), 150 g. of sodium sulfate, 20 g. of sodium acetate, 1.0 g. of 4-hydroxyphthalaldehyde and 20 cc. of formalin (37%); composition J: 5.4 ml. of sulfuric acid (1:1), 150 g. of sodium sulfate, 20 g. of sodium acetate, 1.0 g. of 4-hydroxy-5-methylsophthalaldehyde and 20 cc. of formalin (37%); composition K: 5.4 ml. of sulfuric acid (1:1), 150 g. of sodium sulfate, 20 g. of sodium acetate, 1.0 g. of 4,6-dimethylsophthalaldehyde and 20 cc. of formalin (37%); composition L: 5.4 ml. of sulfuric acid, 150 g. of sodium sulfate, 20 g. of sodium acetate, 1.0 g. of 2,5-dicarboxyterephthalaldehyde and 20 cc. of formalin (37%); composition M: 5.4 ml. of sulfuric acid (1:1), 150 g. of sodium sulfate, 20 g. of sodium acetate, 1.0 g. of 4-sulphoisophthalaldehyde and 20 cc. of formalin (37%).

Each of the compositions was diluted with water to one liter in volume, the pH of which was 4.8.

The developer was a conventional black and white developer for positive film containing metol and hydroquinone and the fixing solution was a conventional acid hardener fixer.

The fog densities of the black and white negative image thus obtained are shown in the following table. The formation of fogs increased slightly in the case of employing phthalaldehyde but such an extent of increase would not affect much on the photographic qualities.

On the other hand, the melting point of the emulsion layers thus processed were measured for knowing the extent of the hardness of the emulsion layers, the results of which are also shown in the same table. This value is the temperature when after washing the film subjected to the hardening processing with water, the emulsion layer was swelled and dissolved in the solution in the case of heating the film to the temperature in an aqueous 0.2 N sodium hydroxide solution.

| Hardening solution | Fog density | Melting point, °C. |
|--------------------|-------------|--------------------|
| A                  | 0.08        | 48.5               |
| B                  | 0.20        | 50.5               |
| C                  | 0.26        | 54.0               |
| D                  | 0.08        | 49.0               |
| E                  | 0.09        | 49.0               |
| F                  | 0.19        | 61.0               |
| G                  | 0.10        | 55.5               |
| H                  | 0.09        | 55.0               |
| I                  | 0.16        | 57.0               |
| J                  | 0.10        | 56.0               |
| K                  | 0.11        | 56.5               |
| L                  | 0.10        | 55.5               |
| M                  | 0.12        | 56.5               |

As shown in the above table, by using formalin and the aromatic dialdehyde simultaneously, the excellent hardening effect which had never been obtained by using each of the aldehydes individually was obtained without being accompanied by an increase in formation of fogs. By the application of the hardening procedure of this invention, the damages to the surface of the emulsion layers of light-sensitive elements when they were processed in an automatic developing machine employing vigorous stirring was remarkably reduced.

#### EXAMPLE 2

After exposing, the gelatino silver halide emulsion layer containing a magenta coupler was subjected to the following reversal color developing procedures: (processing temperature: 30°C.).

| Process:        | Processing time (min.) |
|-----------------|------------------------|
| Hardening       | 1                      |
| Washing         | 1                      |
| 1st development | 3                      |
| Washing         | 0.5                    |

Reversal exposure (uniform exposure at 8000 luxes-sec. over the surface of emulsion layer)

| Process:        | Processing time (min.) |
|-----------------|------------------------|
| 2nd development | 4                      |
| Washing         | 1                      |
| Bleaching       | 1                      |
| Washing         | 0.5                    |
| Fixing          | 1                      |
| Washing         | 1                      |

The composition of the hardening bath was the same in Example 1.

Other compositions for the above-mentioned processings are shown below.

#### Composition for the 1st developer

|                                |      |
|--------------------------------|------|
| N-methyl-p-aminophenol sulfate | 2.0  |
| Sodium sulfite                 | 90.0 |
| Hydroquinone                   | 8.0  |
| Sodium carbonate (monohydrate) | 52.5 |
| Potassium bromide              | 5.0  |
| Potassium thiocyanate          | 1.0  |
| Water to make 1 liter.         |      |

#### Composition for the 2nd developer

|                                                                                |     |     |
|--------------------------------------------------------------------------------|-----|-----|
| Benzyl alcohol                                                                 | ml. | 5.0 |
| Sodium sulfite                                                                 | g.  | 5.0 |
| 3-methyl - 4 - amino-N-ethyl - N - methane - sulfonamide ethyl-aniline sulfate | g.  | 1.5 |
| Potassium bromide                                                              | g.  | 1   |
| Sodium phosphate, tribasic                                                     | g.  | 30  |
| Sodium hydroxide                                                               | g.  | 0.5 |
| Ethylenediamine (aq. 70% soln.)                                                | ml. | 7   |
| Water to make 1 liter.                                                         |     |     |

## 7 Composition for the bleaching bath

|                        |    |     |
|------------------------|----|-----|
| Sodium acetate         | g  | 40  |
| Potassium ferricyanide | g  | 100 |
| Glacial acetic acid    | ml | 20  |
| Potassium bromide      | g  | 30  |
| Water to make 1 liter. |    | 5   |

## Composition for the fixing solution

|                        |   |     |
|------------------------|---|-----|
| Sodium thiosulfate     | g | 150 |
| Sodium acetate         | g | 70  |
| Sodium sulfite         | g | 10  |
| Potassium alum         | g | 20  |
| Water to make 1 liter. |   |     |

The photographic properties of the reversal color images thus obtained are shown in the following table. As shown in the results, the photographic properties were not deteriorated as compared with those obtained without using the dialdehyde and also in some of them, the maximum density was increased. Also, the strength of the emulsion layers processed in accordance with the present invention was very excellent as shown in Example 4.

| Hardening solution | Sensitivity | Maximum density |
|--------------------|-------------|-----------------|
| None               | 1.80        | 2.10            |
| A                  | 1.75        | 2.30            |
| B                  | 1.75        | 2.30            |
| C                  | 1.80        | 2.00            |
| D                  | 1.80        | 2.80            |
| E                  | 1.80        | 2.85            |
| F                  | 1.80        | 2.00            |
| G                  | 1.80        | 2.75            |
| H                  | 1.80        | 2.90            |
| I                  | 1.75        | 2.30            |
| J                  | 1.80        | 2.75            |
| K                  | 1.80        | 2.70            |
| L                  | 1.80        | 2.75            |
| M                  | 1.75        | 2.65            |

## EXAMPLE 3

After exposure, a reversal color photographic light-sensitive film having a light-sensitive emulsion layer containing a commercially-available coupler was processed as in Example 2 except that the following compositions were employed as the hardening solutions.

| Sodium                   | A   | B   | C   | D   |
|--------------------------|-----|-----|-----|-----|
| Sodium sulfate, g.       | 200 | 200 | 200 | 200 |
| Sodium acetate, g.       | 20  | 20  | 20  | 20  |
| Potassium iodide, ml.    | 20  | 20  | 20  | 20  |
| Potassium bromide, g.    | 2.3 | 2.3 | 2.3 | 2.3 |
| Formalin (37%), ml.      | 15  | 15  | 15  | 15  |
| Isophthalaldehyde, g.    |     | 1.0 | 1.0 |     |
| Water to make one liter. |     |     |     |     |

NOTE.—The pH was 4.8.

The results showed that the photographic properties of the sample processed using hardening solution D were same as those of a sample processed using hardening solution A. On the other hand, the strength of the emulsion layer of the sample processed by using hardening solution D was higher than those samples processed by using hardening solution B and hardening solution C respectively as shown in the following table.

| Hardening solution: | Melting point, °C. |
|---------------------|--------------------|
| A                   | 57.0               |
| B                   | 58.5               |
| C                   | 58.5               |
| D                   | 63.0               |

## EXAMPLE 4

After exposing, a gelatino silver halide emulsion layer was subjected to the following photographic processings:

| Process:  | Processing time (min.) |
|-----------|------------------------|
| Hardening | 2                      |
| Fixing    | 1.5                    |
| Washing   | 1.5                    |

The processes were carried out at 35° C. The composition of the developer was as follows, while the fixing solution was a usual acid fixing solution.

| Composition for the developer      | A   | B   |
|------------------------------------|-----|-----|
| N-methyl-p-aminophenol sulfate, g. | 4.5 | 4.5 |
| Sodium carbonate (monohydrate), g. | 41  | 41  |
| Sodium sulfite, g.                 | 15  | 15  |
| Hydroquinone, g.                   | 8.0 | 8.0 |
| Potassium bromide, g.              | 3.0 | 3.0 |
| 6-nitrobenzimidazole, g.           | 0.1 | 0.1 |
| Formaldehyde (37%), ml.            | 2   |     |
| 2-methyl-terephthalaldehyde, g.    | 0.5 |     |
| Sodium hydroxide, g.               | 0.1 | 0.1 |
| Sodium sulfate, g.                 | 40  | 40  |
| Water to make one liter.           |     |     |

The processes were conducted in an automatic developing machine with stirring vigorously. After the processings, the formation of mechanical damage to the surface of the emulsion layer was detected. This showed that the damage in the case of using hardening solution A was reduced to 1/2 of the damage in the case of using hardening solution B. The fog density was 0.10 in both cases.

What is claimed is:

1. In a process for hardening a silver halide photographic light-sensitive element, the improvement which comprises processing the light-sensitive element in a processing bath containing formaldehyde and an aromatic dialdehyde selected from the group consisting of phthalaldehyde, isophthalaldehyde, terephthalaldehyde, 2-methylterephthalaldehyde, 4-hydroxyisophthalaldehyde, 4-hydroxyphthalaldehyde, 5-methylisophthalaldehyde, 2-hydroxyisophthalaldehyde, 4-hydroxyisophthalaldehyde, 4,6-dihydroxyisophthalaldehyde, 4,5-dihydroxyisophthalaldehyde, 4-hydroxy-5-methylisophthalaldehyde, 2-hydroxy-5-methylisophthalaldehyde, 4,6-dimethylisophthalaldehyde, 2,5-dihydroxyterephthalaldehyde, 4,6-dihydroxyisophthalaldehyde, 2,5-dicarboxyterephthalaldehyde and 4-sulfoisophthalaldehyde,

said aromatic dialdehyde capable of maintaining a group capable of increasing water solubility on the aromatic nucleus, said group being a member selected from the group consisting of  $\text{SO}_3\text{H}$ ,  $\text{COOH}$ ,  $\text{OH}$ , and the  $\text{Na}$ ,  $\text{K}$ , or  $\text{NH}_4$  salt thereof.

2. The process as claimed in claim 1 wherein the amount of the dialdehyde is 0.5-1.5 g. per 5-30 ml. of an aqueous solution of formaldehyde when the concentration of the formaldehyde solution is about 37% by weight.

3. The process as claimed in claim 1 wherein said processing bath is a pre-hardening bath.

4. The process as claimed in claim 1 wherein said processing bath is a developing bath.

5. The process of claim 2 wherein the amount of dialdehyde is 0.5-1.5 g. per 20 ml. of an aqueous solution of formaldehyde when the concentration of the formaldehyde solution is about 37% by weight.

6. The process of claim 1 wherein the pH is 4.8.

## OTHER REFERENCES

## References Cited

Mason, Photographic Processing, pp. 151-152, 185-186.

## UNITED STATES PATENTS

|           |         |          |        |    |                                     |
|-----------|---------|----------|--------|----|-------------------------------------|
| 3,565,632 | 2/1971  | Mills    | 96-111 | 5  | NORMAN G. TORCHIN, Primary Examiner |
| 2,629,659 | 2/1953  | Mueller  | 96-111 |    | M. F. KELLEY, Assistant Examiner    |
| 3,102,811 | 9/1963  | Barney   | 96-48  |    |                                     |
| 3,168,400 | 2/1965  | Blackmer | 96-56  |    | U.S. Cl. X.R.                       |
| 3,451,817 | 6/1969  | Bard     | 96-111 | 10 | 96-50, 61, 66, 111                  |
| 3,220,849 | 11/1965 | Baden    | 96-111 |    |                                     |